

## UNITED STATES PATENT OFFICE

DONALD G. ACKERLY, OF EDGEWOOD BOROUGH, PENNSYLVANIA, ASSIGNOR TO THE UNION SWITCH & SIGNAL COMPANY, OF SWISSVALE, PENNSYLVANIA, A CORPORATION OF PENNSYLVANIA

## MANUFACTURE OF ELECTRICAL RECTIFIERS

No Drawing.

Application filed September 11, 1929. Serial No. 391,985.

My invention relates to the manufacture of electrical rectifiers of the type disclosed and claimed in Letters Patent of the United States, No. 1640335, granted to L. O. Gron-dahl on August 23, 1927.

One object of my invention is the provision of novel and improved means for producing metallic copper on the outer surface of the copper oxide in rectifiers of the type referred to.

I will describe one process embodying my invention, and will then point out the novel features thereof in claims.

A copper blank is first treated to form cuprous oxide thereon. This may be done, for example, by heating the blank in an oxygen atmosphere to a temperature of approximately 1000° centigrade.

The treated blank is then placed in a bath of molten metal to reduce the outer layer of the oxide to copper. This molten metal may, for example, be molten lead, in which case the bath should be at a temperature of 500° C. to 600° C. The purpose of producing the layer of copper on the outer surface of the copper oxide is, of course, to make it possible to readily make electrical contact with the cuprous oxide.

The preferred heat treatment of copper oxide rectifiers involves removing the treated blanks from the oxidizing furnace to a second furnace maintained at approximately 500° to 600° C., and quenching the blanks in water after they have reached approximately the temperature of the second furnace. One reason for maintaining the reducing bath of my invention at 500° to 600° C. is to make this bath serve the purpose also of the second furnace, so that the blanks may be quenched in water directly from the reducing bath.

Although I have herein described only one process of manufacturing electrical rectifiers, it is understood that various changes and modifications may be made therein within the scope of the appended claims without departing from the spirit and scope of my invention.

Having thus described my invention, what I claim is:

1. The process of producing a rectifier unit

which consists in treating a copper blank to form cuprous oxide thereon, and then placing the treated blank in a bath of molten metal to reduce the outer surface of the oxide to copper.

2. The process of producing a rectifier unit which consists in treating a copper blank to form cuprous oxide thereon, and then placing the treated blank in a bath of molten lead to reduce the outer surface of the oxide to copper.

3. The process of producing a rectifier unit which consists in treating a copper blank to form cuprous oxide thereon, and then placing the treated blank in a bath of lead at a temperature of 500° C. to 600° C. to reduce the outer surface of the oxide to copper.

4. The process of producing a rectifier unit which consists in treating a copper blank to form cuprous oxide thereon, placing the treated blank in a bath of molten metal to reduce the outer surface of the oxide to copper, and then quenching the blank.

5. The process of producing a rectifier unit which consists in heating a copper blank to approximately 1000° C. to form cuprous oxide thereon, placing the treated blank in a bath of molten metal maintained at approximately 500° to 600° C. to reduce the outer surface of the oxide to copper, and then quenching the blank.

In testimony whereof I affix my signature.

DONALD G. ACKERLY.

55

60

65

70

75

80

85

90

95

100